

## UNITED STATES PATENT OFFICE.

EMIL SCHLEHAHN, OF ARDMORE, ILLINOIS.

## CASE-HARDENING COMPOUND.

No Drawing.

Application filed January 10, 1923. Serial No. 611,851.

To all whom it may concern:

Be it known that I, EMIL SCHLEHAHN, a citizen of the United States of America, residing at Ardmore, in the county of Cook and State of Illinois, have invented new and useful Improvements in Case-Hardening Compounds, of which the following is a specification.

The invention relates to a process of hardening or case-hardening iron and steel and to a new composition of matter, particularly to a case-hardening compound.

According to the present method in vogue iron or steel is exposed to the chemical reaction of certain ingredients employed whereby to the iron or steel a case is imparted of the desired thickness when the mass is placed in a furnace under a certain pre-determined temperature for a considerable period of time.

An object of the invention is to reduce said time necessary for producing the case so that by way of example a thickness of three sixty-fourths of an inch may be obtained when the necessary temperature is maintained for three quarters of an hour.

It is also an object of the invention to provide a compound which renders it unnecessary to cover up the receptacle in which the articles to be hardened are placed prior to being exposed to heat in a furnace.

With these and other objects in view, the invention comprises certain ingredients hereinafter further described, and more particularly pointed out in the claims.

According to the present invention, leather-charcoal, kainite, ammonium chloride and potassium carbonate are reduced to powdered form. A receptacle suitable for introduction into a furnace to be exposed to heat therein is filled with the powder and the article is placed in the receptacle to be surrounded by the powder. Sufficient powder is introduced into the receptacle so that

approximately a layer of three quarters of an inch surrounds the article. The heat maintained in the furnace is approximately between fifteen hundred and sixteen hundred degrees Fahrenheit, and this heat is maintained for a period of three quarters of an hour, whereupon a case is produced having a thickness of three sixty-fourths of an inch.

A specific example of the ingredients employed is as follows:

|                     | Parts by weight. | 55 |
|---------------------|------------------|----|
| Leather charcoal    | 2                |    |
| Potassium carbonate | 3                |    |
| Ammonium chloride   | 1                |    |
| Kainite             | 1                | 60 |

The articles hardened with a novel case-hardening compound meet every requirement as to strength and hardness. If, of course, heating is continued for a longer period than three quarters of an hour the thickness of the case may be increased.

In the foregoing, specific ingredients have been referred to by way of explanation and not by way of limitation. It is, of course, understood that equivalent ingredients may be employed and I, therefore, do not desire to limit myself except as the state of art renders this necessary.

I claim:

1. A case-hardening compound including leather charcoal, potassium carbonate, ammonium chloride and magnesium sulphate.
2. A case-hardening compound including leather charcoal, potassium carbonate, ammonium chloride and kainite.
3. A case-hardening compound including two parts by weight of leather charcoal, three parts by weight of potassium carbonate, one part by weight of ammonium chloride, and one part by weight of kainite.

In witness whereof I affix my signature.

EMIL SCHLEHAHN.